

April 12, 1949.

L. G. HENNING ET AL

2,466,808

PROCESS FOR MAKING CORD

Filed Jan. 29, 1947



INVENTORS:  
LESLIE G. HENNING  
AND  
FRANK L. SESSIONS

or *Frank L. Sessions*

ATTORNEY

## UNITED STATES PATENT OFFICE

2,466,808

## PROCESS FOR MAKING CORD

Leslie G. Henning, Cleveland, and Frank L. Sessions, Lakewood, Ohio; said Henning assignor to said Sessions

Application January 29, 1947, Serial No. 725,118

11 Claims. (Cl. 117—7)

**1**  
This invention relates to improvements in textile cords or the like and processes of making and treating them. Briefly, it relates to the making and treatment of cords, which are made of cotton or other vegetable staple fiber yarns, to improve their strengths, elastic characteristics, toughness and durability, and increase their ability to withstand high, dry temperature without injurious effects.

In our patent application, Serial No. 548,378, filed August 7, 1944, entitled "Textile cord and process of making it," we have described and claimed textile, staple fiber cord and a process of making it which includes certain yarn, thread and cord constructions and twisting operations and wet-stretching and dry-setting of the finished cord at a prescribed stretched length.

In carrying out our present invention we prefer to treat cords that have been made in accordance with the teachings of our above mentioned patent application, although our tests indicate that any staple fiber cotton cord that has not been treated to make it impervious to moisture, may be improved by subjecting it to the process steps herein described.

By our present invention, staple fiber cotton cord is subjected to processing operations as described in the following numbered paragraphs.

*Treatment of cord*

(1) A completely twisted cord is immersed in an aqueous wetting and/or shrinking liquid, or an aqueous wetting, shrinking and impregnating liquid solution wherein it is thoroughly wet, and saturated or soaked. Preferably the cord, while it is in a slack, contractile state, without substantial tension is allowed to shrink in the solution until the cord becomes limp and inert. The liquid solution may also contain a penetrant or wetting agent. It may also contain heat decomposable impregnating and/or curing material, preferably urea, or urea and hexamethylenetetramine, and sulphonated esters of dicarboxylic acids, and, if desired, an accelerator preferably composed of about seven and one-half (7½) parts of diammmonium acid phosphate and one (1) part of hexamethylenetetramine, such chemicals being decomposed or transformed at the temperature to which the cord is to be subsequently subjected as described in paragraph (3) below.

(2) The shrunken, saturated cord resulting from operation (1) is wet-stretched to a length between about 85 per cent and about 96 per cent of the length of the original singles yarns which

were embodied in the cord, and the wet-stretched cord is dried while being prevented from contracting from its stretched length. During this drying operation the temperature should be kept 5 below the curing temperature [described in paragraph (5) below] if the wetting solution contained decomposable materials.

(3) The dry-set cord resulting from the wet-shrinking, impregnating, wet-stretching and dry-setting, operations described in the above paragraphs (1) and (2), is heat-shrunk or heat-shrunk and heat cured if the wet-shrinking and wet-stretching solution also contained heat-decomposable, impregnating, curing material. The 10 temperature for this shrinking and curing heat treatment is above about eighty degrees (80°) centigrade and preferably is about one hundred forty degrees (140°) centigrade. The heat treatment should be carried out while the cord is without 15 substantial tension and is in a slack, contractile state, for the time found necessary to heat-shrink or heat-shrink and heat-cure the cord, but not long enough to scorch or otherwise damage it. Higher temperature demands shorter time.

20 The accompanying drawing shows, diagrammatically, means for progressively and continuously performing the operation of our process.

A clear understanding of the drawings can best be had by referring to the above three numbered paragraphs (1), (2) and (3) under the caption "Treatment of cord."

Fig. 1 of the drawing is a schematic diagram of the entire apparatus; and Fig. 2 is a side view of conical stretching rolls H—H, this view being taken from the plane indicated by line 2, 2, in 35 Fig. 1.

In the drawing, the cord is designated by the reference letter A. It is drawn from the supply reel B by cord-driving rolls C—C. The reel B is provided with an adjustable hub brake D for varying the tension upon the cord. The rolls C may be driven by an electric motor E, the speed of which may be varied by a motor starting and speed controlling rheostat F or other suitable means. The cord A is delivered by rolls C into the wetting and shrinking or wetting, shrinking and impregnating solution contained in the tank G. It passes through the liquid solution in the tank G in a slack, contractile state 40 and is withdrawn by the conical, stretching rolls H—H, which may be driven by an electric motor I, the speed of which may be varied by a motor starting and speed controlling rheostat J or other suitable means.

55 Since the length of the cord contracts as it

passes through the liquid solution in the tank G, the cord must be withdrawn from the tank at a slower speed than that at which it is delivered into it. The delivery and withdrawal speeds of the cord may readily be adjusted so as to keep the cord in the desired slack contractile state while being shrunk in passing through the liquid solution. After being stretched to the desired length, the cord is prevented from contracting while it is being drawn through the drying oven K by the cord-driving rolls L—L and is dried by hot, dry air which may be heated in the stove M and blown through the oven K by the blower N. The rolls L—L, are also driven by the electric motor I at the peripheral speed that is required to keep the tension of the cord substantially constant in its passage through the drying oven so that the cord will be dry-set at substantially the desired stretched length when it emerges from the oven, drawn by the rolls L—L.

From the rolls L—L, the cord is delivered substantially in a slack contractile state into the heat-shrinking and heat-curing oven O and, since the length of the cord contracts as it passes through the heated oven the cord must be withdrawn from the oven at a slower speed than that at which it is delivered into it. The cord-delivery rolls P—P may be driven by an electric motor, Q, the speed of which may be controlled by a motor starting and speed controlling rheostat R. Thus the speed of the cord may be adjusted so that the cord will be allowed to shrink while passing through the oven.

From the cord-delivery rolls P—P the finished cord may be delivered to and wound upon a suitable spool or container S upon which it is preferably wound under uniform light tension limited by a friction slip clutch.

It will be understood that some of the operations may be performed in separate apparatus, operated and controlled entirely independently of the apparatus used for performing others of the operations. For instance, the wet-shrinking, wet-stretching and dry-setting operations may be performed continuously in one apparatus and the dry-set cord instead of being delivered directly to the heat-shrinking and heat-curing apparatus, may be spooled for storage before the heat-shrinking or heat-shrinking and heat-curing operations are performed in independently driven and controlled apparatus.

If desired the cord after being heat-shrunk in oven O, may be wound under a light tension upon a cone or container and be further heat-cured by electronic or other heat-treatment.

The time for which the cord may be subjected to a given high temperature for being shrunk and/or cured without injury, depends upon the construction of the cord, the kind of material of which it is made, the composition of the liquid in which it was shrunk, or, shrunk and impregnated, and the atmospheric conditions to which the cord is subjected in the oven. We have found that staple fiber cotton cord after being shrunk in clear water, wet-stretched and dry-set in the manner described in the above paragraphs (1) and (2) will be heat-shrunk by being subjected for about a minute to a temperature of about 140° centigrade. Such a cord will not be injured if it is subjected to such a temperature for hours or is subjected to higher temperatures for short periods.

Our tests have shown that the resulting elastic characteristics a cord will have after it has been heat-shrunk or heat-shrunk and heat-cured as

described in the above paragraph (3) depend upon the ratio which the length of the wet-stretched, dry-set cord of the above paragraph (2) bears to the length of the original singles yarns embodied in the cord. In general, the elongation of the finished heat-shrunk or heat-shrunk and heat-cured cord at a given intermediate load will be greater, and its breaking strength will be less if the wet-stretching and dry-setting operations performed upon it have resulted in the length of the dry-set cord being relatively low in the range of stretched lengths prescribed in the above paragraph (2), to wit, "between about eighty-five per cent (85%) and about ninety-six per cent (96%) of the length of the original singles yarns embodied in the cord," than they will be if these operations have resulted in the length of the cord being in a higher part of the prescribed range. The length at which the cord should be dry-set in order that it shall have desired stress-strain characteristics after being heat-shrunk and heat-cured may be established readily by trial and test.

While cord that has been shrunk in clear water, wet-stretched, and dry-set as above described in paragraphs (1) and (2) is further improved by the heat-shrinking operation which is described in paragraph (3), our tests indicate that when a liquid wetting, shrinking and curing solution containing urea has been used, the cord's strength, elasticity and ability to withstand high temperature are greatly increased. It appears that the urea in solution impregnates the lumens of the fibers of the cord and that when the urea-impregnated dry-set cord is subjected to a temperature above about one hundred thirty degrees (130°) centigrade the urea is decomposed, certain gases being driven off, leaving in the lumens a residue of higher temperature resisting material. In any event, the cord is improved and becomes stronger, more elastic and more heat resistant than cord which has been shrunk in clear water. Still greater strength, elasticity and ability to withstand high temperature result from the use of urea and hexamethylenetetramine in the solution.

We have been unable to determine whether the urea or hexamethylenetetramine have chemically united with the cellulose of the fiber, but whatever the cause, the cords and consequently the fibers which compose them are greatly improved by the treatment described in the above paragraphs (1), (2) and (3).

Our test indicates that a solution of urea and hexamethylenetetramine in the proportions of about ten pounds, dry weight, of urea; about eight pounds, dry weight of hexamethylenetetramine; about sixteen (16) grams, dry weight, of sulphonated esters of dicarboxylic acids; and about sixteen hundred (1600) grains of an accelerator composed of seven and one-half (7½) parts of diammonium acid phosphate and one (1) part of hexamethylenetetramine, all dissolved in about seven gallons of water, is a superior lubricating liquid solution for wet-twisting threads and cords and for wet-shrinking and impregnating cords before they are wet-stretched and dry-set for heat-shrinking and curing. The shrinking and impregnating effect of this solution on cotton cord and its fibers, respectively, is extremely rapid and complete.

The best results are assured when the yarns are saturated for wet-twisting into thread, the threads are saturated for wet-twisting into cord,

and the complete cord is then processed as described in paragraphs (1), (2) and (3).

Cords which have been processed as described in paragraphs (1) and (2) are substantially benefited by the heat-shrinking and heat-curing operations described in paragraph (3).

The following are data of actual tests that we have made of some staple fiber cotton cords that were treated by our process and of other cords that were not treated by our process. The tests were all made upon a Scott 50 pound capacity "single strand testing machine." They provide a convenient means for comparing critical characteristics of the cords whose data are given. The marked improvement in breaking strength and uniformity of elongation effected by our process are clearly shown by these test results.

in a liquid solution of impregnating and curing material, stretching it while wet to a length between about 85% and about 96% of the length of the original singles yarns embodied in the cord, drying the cord at its stretched length but not further stretching it and heat-shrinking and curing it without substantial tension at a temperature above about 80° centigrade but short of the scorching temperature, for such time that the cord will be heat-shrunk and cured.

4. The process of treating textile natural vegetable staple fiber cord which includes shrinking and impregnating it without substantial tension in a liquid solution containing urea, stretching the shrunken cord while wet, drying it at its stretched length, but not further stretching it, and heat-shrinking and heat-curing it without

| Sample No. | Cord and treatment                                                                                                                                                                                                                                                                                                                                                                                         | Kind of cotton and staple length                     | Elongation at |          | Breaking strength |
|------------|------------------------------------------------------------------------------------------------------------------------------------------------------------------------------------------------------------------------------------------------------------------------------------------------------------------------------------------------------------------------------------------------------------|------------------------------------------------------|---------------|----------|-------------------|
|            |                                                                                                                                                                                                                                                                                                                                                                                                            |                                                      | 10 lbs.       | Break    |                   |
| 0-----     | 22.5/5/3—Water wet-twisted Control Cord.                                                                                                                                                                                                                                                                                                                                                                   | 1 <sup>1</sup> / <sub>2</sub> " Staple Peruvian Pima | Per cent      | Per cent | Lbs.              |
| 1-----     | 22.5/5/3—Water wet-twisted Control Cord, Water wet stretched.                                                                                                                                                                                                                                                                                                                                              | 9.75                                                 | 14.5          | 10       |                   |
| 2-----     | 22.5/5/3—Water wet-twisted Control Cord, Water Shrunk; Water wet-stretched (see Treatment of Cord, paragraphs (1) and (2)); Heat-Shrunk (see Treatment of Cord, paragraph (3)).                                                                                                                                                                                                                            | do                                                   | 3             | 5.5      | 25                |
| 3-----     | 22.5/5/3—Water wet-twisted Control Cord; Wet-shrunk in Solution "A," Stretched while wet with Solution "A" (see footnote); (see Treatment of Cord, paragraphs (1) and (2); Heat-Shrunk (see Treatment of Cord, paragraph (3)).                                                                                                                                                                             | do                                                   | 5.5           | 8.25     | 27.5              |
| 4-----     | 22.5/5/3 Cord—Twisted wet with about 30 per cent aqueous solution of Urea. Wet-shrunk in same strength urea solution; Stretched while wet with same urea solution (see Treatment of Cord, paragraphs (1) and (2)); Heat-Shrunk (see Treatment of Cord, paragraph (3)).                                                                                                                                     | do                                                   | 4.5           | 7.5      | 30                |
| 5-----     | 22.5/5/3 Cord—Twisted wet with an aqueous solution containing about 22 per cent Urea and about 15.5 per cent Hexamethylenetetramine; Wet-shrunk in same solution; Stretched while wet with same solution (see Treatment of Cord, paragraphs (1) and (2)); Heat-shrunk (see Treatment of Cord, paragraph (3)).                                                                                              | do                                                   | 5             | 8.25     | 29                |
| 6-----     | 22.5/5/3—Cord Twisted wet with an aqueous solution of urea, hexamethylenetetramine, sulphonated esters of dicarboxylic acids and an accelerator composed of about seven and one-half (7 <sup>1</sup> / <sub>2</sub> ) parts of Diammonium Acid Phosphate and one (1) part of hexamethylene-tetramine; (see Treatment of Cord, paragraphs (1) and (2)); Heat-shrunk (see Treatment of Cord, paragraph (3)). | do                                                   | 4.5           | 7        | 29.5              |
|            |                                                                                                                                                                                                                                                                                                                                                                                                            | do                                                   | 5             | 8        | 33.5              |

NOTE: In re. Sample 3—Solution "A" is the same aqueous solution as is used in Sample No. 6.

Although we have described in considerable detail certain preferred procedures and solutions for the treatment of cords of the type described, it will be understood that variations and modifications in the composition of the treating solutions and in the processing steps may be made without departing from our invention. We do not, therefore, wish to be limited to the specific materials and process steps herein described but claim as our invention all embodiments thereof coming within the scope of the appended claims.

We claim:

1. The process of treating textile natural vegetable staple fiber cord which includes shrinking it without substantial tension in a liquid, stretching the shrunken cord while wet; drying it at its stretched length but not further stretching it, and heat-shrinking it without substantial tension at a temperature above about eighty degrees (80°) centigrade.

2. The process of treating textile natural vegetable staple fiber cord which includes impregnating it in a solution of heat-decomposable impregnating and curing material, stretching it while wet, drying it at its stretched length but not further stretching it, and heating and curing it without substantial tension at a temperature at or above that at which said heat-decomposable material is decomposed.

3. The process of treating textile natural vegetable staple fiber cord which includes shrinking and impregnating it without substantial tension

substantial tension at a temperature above about eighty degrees (80°) centigrade for such time that the cord will be heat-shrunk and heat-cured.

5. The process of treating textile natural vegetable staple fiber cord which includes shrinking and impregnating it without substantial tension in a liquid solution containing hexamethylenetetramine, stretching the shrunken cord while wet, drying it at its stretched length but not further stretching it, and heat-shrinking and heat-curing it without substantial tension at a temperature above about eighty degrees (80°) centigrade for such time that the cord will be heat-shrunk and heat-cured.

6. The process of treating textile natural vegetable staple fiber cord which includes shrinking and impregnating it without substantial tension in a liquid solution containing urea and hexamethylene-tetramine, stretching it while wet, drying it at its stretched length but not further stretching it, and heat-shrinking and heat-curing

65 it without substantial tension at a temperature above about eighty degrees (80°) centigrade and below the cord-scorching temperature for such time that the cord will be heat-shrunk and heat-cured.

7. The process defined by claim 6 in which the liquid solution contains urea and hexamethylenetetramine in the proportions of about ten pounds, dry weight, of urea, about eight pounds, dry weight, of hexamethylenetetramine and about one gram, dry weight, of a penetrant or

wetting agent such as sulphonated esters of dicarboxylic acids all dissolved in about seven gallons of water.

8. The process of making textile natural vegetable staple fiber cord as defined by claim 6 in which the liquid solution contains urea and hexamethylenetetramine in the proportions of about ten pounds, dry weight, of urea, about eight pounds, dry weight, of hexamethylene tetramine, about sixteen (16) grams dry weight, of a penetrant or wetting agent such as sulphonated esters of dicarboxylic acids, and about sixteen hundred (1600) grains of an accelerator such as one composed of seven and one-half (7½) parts of diammonium acid phosphate to one (1) part of hexamethylenetetramine, all dissolved in about seven gallons of water.

9. The process of treating textile natural vegetable staple fiber cord made of a plurality of original singles yarns of known length, which includes saturating and shrinking the cord in liquid while the cord is in a slack, contractile state; wet-stretching the wet-shrunken cord to a length between about eighty-five per cent (85%) and ninety-six per cent (96%) of the length of the original singles yarns embodied in the cord; drying the cord while it is being prevented from contracting from its stretched length; releasing the stretching tension; and heat-shrinking the dried cord at a temperature above about eighty degrees (80°) C., but below the cord-scorching temperature while the cord is in a slack, contractile state.

10. The process of treating textile natural vegetable staple fiber cord made of a plurality of original singles yarns of known length, which includes saturating and shrinking the cord in a liquid solution containing heat-decomposable, impregnating, curing material while the cord is in a slack, contractile state; wet-stretching the shrunken cord to a length between about eighty-five per cent (85%) and ninety-six per cent (96%) of the original singles yarns embodied in

5 the cord; drying the cord while it is being prevented from contracting from its stretched length; releasing the stretching tension; and heat-shrinking and heat-curing the dried cord at a temperature above about eighty degrees (80°) C., but below the cord-scorching temperature while the cord is in a slack, contractile state.

10 11. The process of treating textile natural vegetable staple fiber cord which includes (1) thoroughly wetting it in an aqueous wetting, shrinking and impregnating liquid solution; (2) allowing the cord to shrink while it is in a slack contractile state without tension while in the solution until the cord becomes limp and inert; (3) 15 wet-stretching the shrunken cord resulting from operations (1) and (2) to a length between about eighty-five per cent (85%) and ninety-six per cent (96%) of the length of the original singles yarns which were embodied in the cord; (4) 20 drying the wet-stretched cord while it is prevented from contracting from its stretched length; (5) releasing the stretching tension; and (6) heat curing the released cord at a temperature above about eighty degrees (80°) C. but below the cord-scorching temperature.

LESLIE G. HENNING.  
FRANK L. SESSIONS.

#### REFERENCES CITED

- 30 The following references are of record in the file of this patent:

#### UNITED STATES PATENTS

| Number       | Name             | Date           |
|--------------|------------------|----------------|
| 35 1,852,706 | Eisenstein       | Apr. 5, 1932   |
| 2,121,005    | Bener            | June 21, 1938  |
| 2,173,997    | Burgeni          | Sept. 26, 1939 |
| 2,192,865    | Monsaroff et al. | Mar. 5, 1940   |
| 40 2,220,958 | Jennings         | Nov. 12, 1940  |
| 2,325,060    | Ingersoll        | July 27, 1943  |
| 2,364,467    | Nickerson        | Dec. 5, 1944   |
| 2,381,398    | Bosomworth       | Aug. 7, 1945   |
| 2,398,787    | Hansen et al.    | Apr. 23, 1946  |